# EUROPEAN PATENT APPLICATION

(11) **EP 0 310 202 A1**
(43) Date of publication of application: **05.04.1989**
(21) Application number: 88202163.7
(22) Date of filing: 30.09.1988
(51) Int. Cl.: D02G 3/40, D02G 3/44

(54) **Combinations of polyolefin filaments and yarns of low wetting and adhesive power and filaments and yarns of high wetting and adhesive power**

(30) Priority: 02.10.1987 DE 3733429
(71) Applicant: STAMICARBON B.V., NL-6167 AC Geleen (NL)
(72) Inventor: Bruinink, Peter, NL-6211 BG Maastricht (NL); Hogenboom, Eric Henricus Maria, NL-6222 AK Maastricht (NL)

(57) **Abstract**

The invention relates to combinations of polyolefin filaments and yarns having high tensile strengths and moduli and low wetting and adhesive power in particular in respect of customary matrix materials as used for producing composite articles, and filaments and yarns of good wetting and adhesive power. These combinations combine to good tensile strength and modulus values of polyolefin filaments and yarns with high wettability by and adhesion to customary polymer matrix materials, the wetting and adhesive power being obtainable in a more economical manner than with the previously disclosed coating with coatings which enhance the wetting and adhesive power or with a corona or plasma treatment or a mechanical and/or chemical roughening, which pretreatments also had the effect of impairing the tensile strengths.

## Description

The present invention relates to combinations of polyolefin filaments and yarns having high tensile strengths and moduli and low wetting and adhesive power, in particular in respect of customary matrix materials, and filaments and yarns of high wetting and adhesive power.

Polyolefin filaments and yarns having high tensile strengths and high moduli have very poor wettability by and adhesion to hydrophilic materials, such as heat-curing phenolic, epoxy, vinylester, polyester and acrylate resin based resins customarily used for producing composite materials, and also thermoplastics and rubber. For this reason they are not particularly suitable for producing composite materials without pretreatment.

There have therefore been attempts to improve the wetting and adhesive power by coatings, plasma and corona treatment and also by mechanical and/or chemical roughening. Apart from the fact that such measures are costly, they frequently also bring about a reduction in the tensile-strength properties of the filaments and yarns thus treated.

It is therefore an object of the present invention to provide an inexpensive way of enhancing the wetting and adhesive properties of polyolefin filaments and yarns while retaining their tensile strengths and moduli.

This object is achieved according to the invention by combinations of polyolefin filaments and yarns having high tensile strengths and moduli and low wetting and adhesive power, in particular in respect of customary matrix materials, and filaments and yarns of high wetting and adhesive power.

These combinations can be used in particular for producing composite materials using the aforementioned customary polymeric matrix materials, since they adhere well to the matrix materials without their desired high tensile strength and modulus values having been impaired by a surface treatment.

Preferably the polyolefin filaments and yarns of low wetting and adhesive power are those which have been produced by the gel process and subsequent high drawing. This gel process, which is described for example in DE Offenlegungsschrift 3,724,434 and also in GB-A-2,042,414 and -2,051,667, comprises essentially dissolving a polyolefin in a solvent, moulding the solution at a temperature above the dissolving temperature of the polyolefin into a filament, cooling the filament, for gelling, to a temperature below the dissolving temperature and then drawing the gel filament with solvent removal, preferably employing draw ratios of more than 20, in particular more than 30.

The polyolefins used consist preferably of polyethylenes in particular linear polyethylenes, having an ultrahigh molecular weight of more than 600,000 g/mol (weight average of molecular weight). These polyethylenes may contain minor amounts preferably not more 5 mol %, of one or more other alkenes copolymerizable therewith, such as propylene, butylene, pentene, hexene, 4-methylpentene, octene etc. Preferably the polyethylenes can have from 1 to 10, in particular 2 to 6, methyl or ethyl groups per 1,000 carbon atoms. However, it is also possible to use other polyolefins, for example polypropylene homopolymers and copolymers; furthermore, the polyolefins used may contain minor amounts of one or more other polymers in particular alkene-l-polymers.

It is particularly suitable to use polyolefin filaments having tensile strengths of more than 2 GPa and moduli of more than 60 GPa.

The filaments and yarns of high wetting and adhesive power consist preferably of glass, carbon, polyamides or polyesters. However, it is also possible to resort to other filaments and yarns of high wetting and adhesive power in respect of the abovementioned materials.

Advantageously, the two filament and yarn types are combined by core spinning a filament or yarn of low wetting and adhesive power with a filament and/or a yarn of high wetting and adhesive power, or by twisting the two components.

In general, the proportion of filaments or yarns of high wetting and adhesive power in relation to the proportion of filaments and yarns of low wetting and adhesive power is 10 to 50% by weight, in particular 15 to 30% by weight, particularly advantageously these proportions being about 25% by weight in the case of core spinning and about 15% by weight in the case of twisting. Composite materials which have been produced using combinations according to the invention as reinforcing materials can be used for example to produce sport articles such as tennis rackets or golf clubs, boat hulls such as kayak or canoe boat hulls, antiballistic articles, helmets, high-pressure hoses etc.

## Claims

1. A combination of polyolefin filaments and yarns having high tensile strengths and moduli and low wetting and adhesive power, in particular in respect of customary matrix materials, and filaments and yarns of high wetting and adhesive power.

2. A combination as claimed in claim 1, wherein the polyolefin filaments and yarns of low wetting and adhesive power have been produced by the gel process and been highly drawn.

3. A combination as claimed in either of claims 1 and 2, wherein the polyolefin filaments and yarns consist of polyethylenes, in particular linear polyethylenes, having an ultrahigh molecular weight of more than 600,000 g/mol (weight average of molecular weight).

4. A combination as claimed in any of claims 1 to 3, wherein the filaments and yarns of high wetting and adhesive power consist of glass, carbon, polyesters or polyamides.

5. A combination as claimed in any of claims 1 to 4, wherein the filaments or yarns of low wetting and adhesive power have been combined with filaments or yarns of high wetting and adhesive power by core spinning or twisting.

6. A combination as claimed in any of claims 1 to 5, wherein the proportion of filaments of yarns of high wetting and adhesive power in relation to the proportion of filaments and yarns of low wetting and adhesive power is 10 to 50% by weight, in particular 15 to 30% by weight.

7. Use of a combination as claimed in any of claims 1 to 6 for producing composite materials.
